

# UNITED STATES PATENT OFFICE.

WILLIAM THUM, OF HAMMOND, AND JOHN J. MULLIGAN, OF EAST CHICAGO, INDIANA,  
ASSIGNORS TO UNITED STATES METALS REFINING COMPANY, OF NEW YORK, N. Y.,  
A CORPORATION OF NEW JERSEY.

## METHOD OF ELECTROPLATING.

1,283,973.

Specification of Letters Patent.

Patented Nov. 5, 1918.

No Drawing.

Application filed July 31, 1918. Serial No. 247,640.

*To all whom it may concern:*

Be it known, that we, WILLIAM THUM and JOHN J. MULLIGAN, citizens of the United States, residing at Hammond and East Chicago, respectively, in the county of Lake and State of Indiana, have invented certain new and useful Improvements in Methods of Electroplating; and we do hereby declare the following to be a full, clear, and exact 10 description of the invention, such as will enable others skilled in the art to which it appertains to make and use the same.

The invention relates to electroplating the surfaces of steel, iron, ferrous alloys and 15 kindred base metals belonging to the more electro-positive series of metals, with lead, copper or kindred metals belonging to the more electro-negative series.

The object of the invention is to obtain a 20 homogeneous and firmly adhering deposit of the plating metal directly on the steel, iron or kindred metal surfaces.

To this end the contact reactions (some of 25 which are of a purely chemical or catalytic action) which usually result from the contact of the base metal with the electrolyte containing acids or producing free acids in the process of electrolysis, and which cause such porosity in the shape of pin holes as to 30 render a thin plating useless as a protective covering for the base metal, are prevented by the direct electroplating of the surfaces of the base metal with an initial thin, smooth, homogeneous and adhesive coating 35 of a plating metal such as lead which protects the base metal from contact with the electrolyte during the continued deposition of the plating metal.

While the invention may be employed 40 with advantage in the electrodeposition of various metals on iron, steel and ferrous alloys, it is particularly adapted for the electro-deposition of lead, and its application to lead plating will be specifically described.

The preferred procedure to obtain the 45 desired electro-plated coating is as follows. The surfaces of the articles to be plated are first cleansed of foreign adherences, such as oxids, grease and slags. This cleansing 50 operation may be effected in the usual way by acid and alkaline dips or pickles, but we have found that a sand blast applied in a suitable manner is quite satisfactory for this purpose.

The next step in the process is to warm the 55 thus prepared article to a desired temperature of 90 to 110 degrees Fahrenheit. This operation is preferably done immediately after the cleansing operation so as to avoid any possibility of oxidation or condensation 60 of moisture on the surface to be plated.

The article may then be connected with the source of the depositing current, either by a flexible or rigid conductor, and immediately dipped into a solution of animal gelatin and clean water, which solution is previously prepared by dissolving the gelatin in the water at a temperature of about 150 degrees F. The percentage of gelatin in the solution can be varied to some extent, but is 70 preferably approximately two per cent. When plating the interior of a container or other article, it is found to be more convenient in some cases to fill the article with the gelatin solution, instead of dipping the article into the solution, or the solution may 75 be applied in other ways.

The temperature of both the article to be plated and the solution is preferably maintained above 90° F. throughout the remaining steps in the process.

The next step, which, to secure the best results, should be performed immediately after the article has been dipped, or after the solution has been emptied from the 85 interior of the article, as the case may be, is to transfer the article to the plating bath or, if the shape of the article permits, it may be filled with the electrolyte. As the article has previously been connected with the electric current, electrolytic action takes place 90 at the moment of contact of the article and electrolyte.

In the plating operation we have found that the use for a short space of time of an 95 initial current of abnormally high density results in the deposit upon the base metal surface of a perfectly homogeneous covering which will build further without porosity after the current density has been lowered 100 to normal.

As a normal current density with moderate circulation of the electrolyte, we have found that 10 to 15 amperes per square foot give satisfactory results. For the initial excessive current density, which need only be applied for a few seconds (less than a minute) we have found that 25 to 50 amperes 105

per square foot is effective in obtaining the desired homogeneous deposit.

The composition of the electrolytes may be the same as ordinarily used in electroplating; for example, when a lead fluosilicate solution is employed, a lead contents of 9 to 11 per cent. and a total hydrofluosilicic acid contents of 10 to 12 per cent. is recommended.

10 In explanation of the assumed reactions taking place during the several steps of the process, it appears evident that the formation of minute gas globules which would otherwise be caused by chemical reaction at 15 the moment of contact of the base metal to be plated and the acid constituents of the electrolyte is prevented by the gelatin solution. It acts as a momentary protective coating against direct contact of the electrolyte, and simultaneously the overpowering electric energy of the excessive current density deposits an initial homogeneous and protective metal coating in the shortest possible interval and before the protective gelatin coating has been fully diffused with the electrolyte wherein it acts as an addition agent to promote a smooth electrodeposit.

When lead is used as the anode, it should preferably be of the highest purity, and it 30 can be cast into any convenient shape to suit the requirements. By rotating or otherwise moving either one of the electrodes, a much increased mixing or circulating of the electrolyte can be brought about, thereby permitting a relative increase in the excessive 35 and normal current densities and consequently an increase in the rate of deposit.

In practising this invention, other compounds containing an addition agent acting 40 similarly to animal gelatin can be used as the initial protective and soluble coating but this will obviously in no way change the principles of the invention.

What is claimed is:—

45 1. The method of electroplating which

consists in covering the surface to be plated with a protective film soluble and diffusible in the electrolyte and then depositing the plating metal thereon by electrolysis.

2. The method of electroplating which 50 consists in covering the surface to be plated with a protective film soluble and diffusible in the electrolyte and then depositing the plating metal thereon by electrolysis with an initial current of abnormally high density, reduced to normal after a short interval.

3. The method of electroplating which 55 consists in covering the surface to be plated with a film of gelatin solution and then depositing the plating metal thereon by electrolysis with an initial current of abnormally high density reduced to normal after a short interval.

4. The method of directly electroplating 60 the surfaces of iron, steel and kindred base metals which consists in covering the surface to be plated with a protective film soluble and diffusible in the electrolyte, subjecting the same to the action of a plating bath current having an abnormally high current density for a short interval, and then reducing the current density to normal until the desired thickness of deposit has been obtained.

5. The method of directly electroplating 75 the surfaces of iron, steel and kindred base metals which consists in covering the surface to be plated with a protective film of gelatin, connecting the article to be plated to the source of electric current, and then subjecting the same to the action of a plating bath current having an abnormally high current density for a short interval, and then reducing the current density to normal until the desired thickness of deposit has been obtained.

WILLIAM THUM.  
JOHN J. MULLIGAN.